

## UNITED STATES PATENT OFFICE

2,570,355

## METAL ALLOY

Sidney Low, Springfield, Mass.

No Drawing. Application April 9, 1949,  
Serial No. 86,589

1 Claim. (Cl. 75—171)

1

My invention relates to improvements in metal alloys and is directed more particularly to a metal alloy which is especially adapted for casting dental bridges and like appliances.

This application is a continuation in part of an application bearing Serial Number 44,595 and filed by me on August 16, 1948, now abandoned.

The principal object of my invention is the provision of a new casting alloy which is adapted for dental appliances and the like, which is highly resistant to corrosion encountered in investments of plaster of Paris and the like, which possesses good ductility enhancing the working characteristics thereof, which has a pleasing color and appearance as well as good machinability, and which has a low melting point of about 2300° F.

The novel features of my invention are accomplished by the combining of certain elements which are selected for their individual characteristics and function and combine for producing an alloy possessing superior properties for the casting of dental bridges and the like.

The alloy of my invention includes elements within the percentage ranges as follows:

|            |            |
|------------|------------|
| Carbon     | 0.50% Max. |
| Manganese  | 2.0% Max.  |
| Silicon    | 2.0% Max.  |
| Nickel     | 50.0—70.0% |
| Chromium   | 10.0—20.0% |
| Copper     | 3.0—20.0%  |
| Molybdenum | 3.0—4.0%   |
| Aluminum   | 0.02—2.0%  |
| Titanium   | 1.0% Max.  |
| Zirconium  | 1.0% Max.  |
| Silver     | 2.0% Max.  |

Carbon is primarily an impurity necessarily tolerated in my alloy. Whenever possible, the carbon content is held to approximately 0.05% as I have found that an increase in the carbon content tends to increase the hardness and strength of the alloy and that it also tends to decrease the ductility and corrosion resistance. I have found that the carbon content should not exceed 0.50% under any conditions.

Manganese serves as an aid to the melting of the alloy. Furthermore, as is well known, manganese is used to "clean up" a melt prior to tapping. It increases the fluidity of the alloy permitting lighter sections to be successfully cast. I have found that the manganese content should not exceed 2.0% under any conditions.

Silicon, as manganese, serves as an aid to the melting of the alloy as well as tone alloying additions. It too is used to "clean up" a melt prior to

2

tapping. Furthermore, it serves to increase the corrosion resistance of the resistant alloy in oxidizing media. As with manganese, silicon serves to increase the fluidity of the alloy permitting lighter sections to be successfully cast. I have found that the silicon content should not exceed 2.0% as a maximum.

Nickel serves as a very excellent base to which the alloying additions may be made. Nickel possesses fair corrosion resistance qualities and a reasonably low melting point. The other alloying additions may be readily added to the nickel base, as will presently be observed, since all are readily soluble in both molten and solid nickel.

If desired, cobalt in like quantity may be substituted for nickel, or these elements may be used in combination with each other within the scope of my invention. Cobalt behaves very similarly to nickel although cobalt bearing alloys are more difficult to machine.

Chromium is added in quantities from 10—20% in order to increase the corrosion resistance of the material. When the chromium content is less than 10%, the material is not corrosion resistant enough, particularly in the weak solutions of lactic acid present in the human mouth. Chromium contents greater than 20% are avoided in order to maintain a reasonably low melting point and to avoid the difficulties of the chromium combining with the sulphur in plaster of Paris bound investments.

In my alloy, I provide a maximum of 20.0% copper whereas other alloys known in the art employ a maximum of 10.0%. In such prior art alloys, the copper content is held below 10.0% to prevent free copper from being thrown from the solution when the alloy solidifies. I have found that copper in the amounts present in these prior art alloys will not prevent the sulphur in gypsum bound investments from combining with the surface of the casting. Furthermore copper in amounts below 20% will increase the corrosion resistance of the alloy in the human mouth.

Likewise, in my alloy, I provide a maximum of 2.0% aluminum whereas other alloys known in the art employ none. I have found that the combination of aluminum and copper in my alloy permits higher copper additions to be made without the subsequent precipitation of free copper. The copper and aluminum must be added in the form of a master alloy shortly to be described as I have found that additions of metallic copper and aluminum will not result in the desired alloy.

Molybdenum is used to increase the corrosion resistance. I have found that a maximum of 4.0% of molybdenum should not be exceeded.

Furthermore, my alloy contains titanium, zirconium and silver whereas other alloys known in the art employ none.

Titanium is used to increase the strength and hardness, which aluminum also does, whereas in prior art alloys the carbon supplies the hardness and strength. I have found that the titanium content should not exceed 1.0%.

Zirconium is also used to increase the strength and hardness as compared with the carbon alloys of other known types. I have found that the zirconium content should not exceed 1.0%.

The silver is added to further enhance its corrosion resistance. I have found that the silver content should not exceed 2.0%.

A minimum of iron is desired so that none is intentionally included. Iron would react unfavorably with any sulphur present in the investment in which the alloy is cast and would tend to raise the melting point both of which are objectionable features.

Particularly desirable results have been obtained where the proportions are as follows:

|            |            |
|------------|------------|
| Carbon     | 0.05% Max. |
| Manganese  | 0.60% Max. |
| Silicon    | 0.60% Max. |
| Nickel     | 55.0-62.0% |
| Chromium   | 14.0-17.0% |
| Copper     | 13.0-20.0% |
| Molybdenum | 3.0-4.0%   |
| Aluminum   | 0.02-0.10% |
| Titanium   | 0.40-0.60% |
| Zirconium  | 0.40-0.60% |
| Silver     | 0.60-0.80% |

More specifically, the proportions as follows provide an alloy which is easily and readily usable for producing dental bridges and the like:

|            |         |
|------------|---------|
|            | Percent |
| Carbon     | 0.20    |
| Manganese  | 0.60    |
| Silicon    | 0.60    |
| Nickel     | 56.0    |
| Chromium   | 13.0    |
| Copper     | 17.0    |
| Molybdenum | 3.0     |
| Aluminum   | 0.10    |
| Titanium   | 0.50    |
| Zirconium  | 0.50    |
| Silver     | 0.70    |

The alloy is high in copper and aluminum and has very marked resistance to the action of sulphur which is present in the usual investments in which castings are made. Plaster of Paris is an ordinary material used for investments.

Also, the alloy is very low in iron which is necessary to overcome corrosion and hold the melting point below a range where expensive and complicating equipment must be used.

Castings made from the alloy when taken from the mold have a pleasingly bright and clean appearance, are ductile, and possess good machineability.

The combination of elements provide a casting having an outer layer or skin which is rich in copper and aluminum, which is desired for its resistance to sulphur attack in the mold. This skin is only a few millionths of an inch thick and is subsequently polished off.

The elements in the specific proportions provide an alloy which has a low melting point of

about 2300° F. to facilitate ready and easy casting in ordinary investments, presents a brilliant appearance, has marked resistance to corrosion, and possesses a very desirable ductility and machineability.

The base composition used for producing my alloy comprises:

|           |             |
|-----------|-------------|
| Carbon    | 0.05% Max.  |
| Manganese | 0.60% Max.  |
| Silicon   | 0.60% Max.  |
| Chromium  | 14.0-17.0%  |
| Copper    | 13.0-20.0%  |
| Aluminum  | 0.02-0.10%  |
| Nickel    | The balance |

This base composition has uses in itself. It may be used in wire for resistance furnaces containing a sulphur bearing atmosphere as it has a high resistance to sulphur attack.

The "as cast" tensile properties of this base composition are:

|                   |                            |
|-------------------|----------------------------|
| Tensile strength  | 80,000-90,000 p. s. i.     |
| Yield point       | 55,000-60,000 p. s. i.     |
| Elongation        | 15-20%                     |
| Reduction of area | 25-35%                     |
| Hardness          | approximately 120 B. H. N. |

The copper and aluminum must be added in the form of a master alloy addition of the following composition:

|          |           |
|----------|-----------|
| Aluminum | 9.0-11.0% |
| Iron     | 0.90-1.0% |
| Copper   | balance   |

If the copper addition is not made in this manner, there is a marked change in the properties of the resultant alloy. Additions of metallic copper and aluminum will not result in the desired alloy.

An alloy, having the same nominal composition, but with the copper and aluminum additions of each separate metal will be hard and brittle. Furthermore, free copper will be thrown out of solution in the form of small nodules of copper.

When the additions of the master alloy of copper, aluminum, and iron are made, suitable allowances must be made for oxidation losses. A master alloy addition of 17.0% copper plus 1.7% aluminum will result in a residual copper and aluminum of approximately 16% and 0.05% respectively.

While the base metal composition possesses unique and valuable properties, it is generally too soft and ductile for dental usage. Other alloying elements such as molybdenum, titanium, zirconium and silver are usually added to both further enhance its corrosion resistance, strength and hardness.

The hardness and strength may also be further increased by the addition of more aluminum either by itself or in the form of a master alloy such as nickel-aluminum.

The control of hardness and strength may also be effected by the use of a so-called "hardener" melt having nominally the same composition as the "base" melt except that the aluminum and copper are added separately. Suitable combinations of "hardener" and "base" melts may then be made to procure any desired hardness. Oxidation that occurs during the melting together of these two types of melts will insure that no free copper will be thrown out of solution upon subsequent solidification of the combined melts.

The invention may be embodied in other specific forms without departing from the essen-

tial characteristics thereof. Hence, the present embodiments are therefore to be considered in all respects merely as being illustrative and not as being restrictive, the scope of the invention being indicated by the appended claims rather than by the foregoing description, and all modifications and variations as fall within the meaning and purview and range of equivalency of the appended claim are therefore intended to be embraced therein.

What it is desired to claim and secure by Letters Patent of the United States is:

A corrosion resistant casting alloy for dentures consisting of elements having proportions as follows: carbon no more than 0.05%; manganese no more than 0.60%; silicon no more than 0.60%; nickel between 55.0% and 62.0%; chromium between 14.0% and 17.0%; copper between 13.0% and 20.0%; molybdenum between 3.0% and 4.0%; aluminum between 0.02% and 0.10%; titanium 20 between 0.40% and 0.60%; zirconium between

0.40% and 0.60%; silver between 0.60% and 0.80%.

SIDNEY LOW.

#### REFERENCES CITED

The following references are of record in the file of this patent:

#### UNITED STATES PATENTS

| 10 | Number    | Name       | Date          |
|----|-----------|------------|---------------|
|    | 1,115,239 | Parr       | Oct. 27, 1914 |
|    | 1,838,130 | Beckinsale | Dec. 29, 1931 |
|    | 2,309,136 | Neiman     | Jan. 26, 1943 |

#### FOREIGN PATENTS

| 15 | Number            | Country       | Date           |
|----|-------------------|---------------|----------------|
|    | 255,919           | Germany       | Jan. 23, 1913  |
|    | 256,361           | Germany       | Feb. 6, 1913   |
|    | 265,076           | Germany       | Sept. 30, 1913 |
|    | 18,212<br>of 1913 | Great Britain | July 9, 1914   |